# EUROPEAN PATENT SPECIFICATION

(11) **EP 1 927 666 B1**
(45) Date of publication and mention of the grant of the patent: **24.04.2013**
(21) Application number: 05801995.1
(22) Date of filing: 02.11.2005
(51) Int. Cl.: C21B 5/02, C21B 3/02, C22C 38/08

(54) **A SMELTING PROCESS OF FERRONICKEL WITH NICKEL OXIDE ORE CONTAINING OF CRYSTAL WATER IN A BLAST FURNACE**
VERHÜTTUNGSVERFAHREN FÜR FERRONICKEL MIT KRISTALLWASSER ENTHALTENDEM NICKELOXIDERZ IN EINEM HOCHOFEN
PROCÉDÉ DE FABRICATION DE FERRONICKEL PAR FUSION DE MINERAI D OXYDE DE NICKEL CONTENANT DES CRISTAUX D'EAU DANS UN HAUT-FOURNEAU

(30) Priority: 16.09.2005 CN 200510102985
(43) Date of publication of application: 04.06.2008
(73) Proprietor: Liu, Shenjie, Tongjun Tonglu Zhejiang 311-500 (CN)
(72) Inventor: Liu, Shenjie, Tongjun Tonglu Zhejiang 311-500 (CN)
(74) Representative: Gervasi, Gemma
(86) International application number: PCT/CN2005/001828
(87) International publication number: WO 2006/045254

(56) References cited:
- CN-A- 1 205 743
- CN-A- 1 603 439
- GB-A- 1 400 505
- JP-A- 62 290 843
- JP-A- 2001 303 113
- RU-C1- 2 132 400
- RU-C1- 2 157 412
- US-A- 3 746 533
- ZHENMIN XIAO.: 'STATUS OF EXPLOTATION OF LATERITE TYPE NICKEL ORE AND APPLICATIONS OF HIGH PRESSURE ACID LEACHING TECHNOLOGY IN THE WORLD.' CHINESE MINING. vol. 11, no. 1, XP008099211

## Description

### Technical field

The present invention relates to a method of blast-furnace smelting, more particularly to a metallurgical method of ferronickel production by blast-furnace smelting nickel oxide ore with crystal water.

### Background of the invention

Global extensive uses of stainless steel and special steel lead to supply shortage and rapid rise in price of nickel metal, a main element used to smelt stainless steel and special steel. Conventional technology is mature that nickel metal is produced by mainly extracting from nickel sulfide ore, which covers 30% of the nickel resources on the earth. But at present, reserves are in shortage and resources are in crises after continuous exploitation for nearly one century. People have to pay more attention to the extraction of nickel metal from laterite nickel ore (nickel oxide ore) covering 70% of nickel resources on the earth. The main reason that laterite nickel ore hasn't been exploited on a large scale for a long time is that the technology extracting Ni from such mineral resources is characterized by high cost, technological complexity, low yield, severe pollution. At present, for high-grade laterite nickel ore (nickel content above 2.0%), ore-smelting furnace is generally used to smelt on the international, however, this method is provided with disadvantages such as high power consumption, severe environmental pollution and low yield of intermittent production. For low-grade laterite nickel ore, hydrometallurgy is commonly used, namely, a method of vitriol soaking, i.e. converting solid-state nickel oxide, chromic oxide, ferric oxide or the like in the laterite nickel ore to mixed solution of liquid-state nickel sulfate, chrome sulfate, iron sulfate (Fe²⁺) and the like, then separating nickel sulfate thereby, forming nickel metal only accounting for 1-2% of the gross by electrolysis with all the other components wasted. The process equipment is characterized by large one-off investment, complex process, long periodicity, severe environmental pollution. Blast-furnace smelting may also be used, however, because Cr₂O₃ as concomitant commonly exists in laterite nickel ore, extremely high melting point of its own can lead to large viscosity of molten iron so that molten iron containing nickel and chrome can't flow out successfully and cause severe results such as frozen furnace and damaged furnace. Many corporations and research organizations at home and abroad have studied the technology for a long time that ferronickel (nickel iron) can be obtained by blast-furnace smelting laterite nickel ore in one-step way, but hitherto no success is reported.

Patent RU 2,157,412 C1 discloses a metallurgical method of ferronickel production by blast-furnace including the preparation of ore, production of sinter and its charging into furnace together with coke, supply of heated air blast and discharge of heat products; in this method, prior to sintering, ore is mixed with hot nickel sinter and fluxed up to basicity CaO/SiO2=0.4-0.6, and Fe/Ni ratio is maintained within 6-12; fluorite is not used in the method of this document.

Patent application JP 58-213837 A discloses a metallurgical method to obtain sintering of chrome in short-time, by blending fine chrome ore, coke breeze and return ore as principal starting materials with suitable amounts of secondary starting materials such as powdered limestone and silica sand, and possibly fluorite, to prepare a starting material to be sintered.

Consequently, it is urgent problem to be solved in this business to find an industrial method that nickel iron is smelted directly from laterite nickel ore, which is characterized by high efficiency, low consumption, high yield, low cost and no pollution or little pollution.

### Summary of the invention

To solve the above problem, the present invention provides a metallurgical method of ferronickel by blast-furnace smelting nickel oxide ore containing crystal water in one-step way.

The above inventive object is achieved by the following technical proposal.

The invention provides a metallurgical method of ferronickel production according to claim 1.

The metallurgical method of ferronickel production by blast-furnace smelting nickel oxide ore with crystal water in the present invention further includes the following steps:
Crushing and sieving the sintered blocks obtained by first sintering by means of a sieve with openings in the range between 25 and 53 µm (300-500 meshes), and then producing refined ore powder by magnetic sorting;
Mixing the feed of the refined ore powder with coke powder, calcium lime/limestone and sintering to obtain sintered ore blocks;
Mixing the sintered ore blocks obtained by second sintering with coke, lime/limestone, dolomite and fluorite, and then blast-furnace smelting to obtain ferronickel.

Wherein the preferable weight ratio of the additives to the sintered ore is:

| | |
|---|---|
| fluorite | 0.3 ∼ 10% |
| dolomite | 0.5 ∼ 5% |
| limestone/calcium lime | 8 ∼ 20%. |

Wherein the content of CaO in limestone is greater than 50%, while that of CaO in calcium lime is greater than 80%; the content of Mg in the dolomite is higher than 10% and that of CaF₂ in fluorite is bigger than 80%.

Compared with the prior art, furnace temperature can reach up to about 1700 °C in the conventional blast-furnace smelting technology, chrome contained in nickel oxide ore mainly exists in the form of Cr₂O₃ whose melting point is about 2300° C, consequently, the reduction degree of chrome in nickel oxide ore is limited to cause bad fluidity of the obtained molten iron and easily to produce phenomenon of frozen furnace, and even result in accidents. In metallurgical method of ferronickel production by smelting nickel and chrome iron ore provided by the present invention, the addition of fluorite can lower the influence of chrome on furnace temperature effectively and raise the fluidity of molten iron, meanwhile, because the addition quantity of fluorite in metallurgical method provided by the present invention is strictly calculated, the accidents, such as burnout of the crucible, caused by too high addition quantity of fluorite, can be effectively avoided. In the metallurgical method provided by the present invention, meanwhile, magnesium contained in dolomite may also be helpful to solve the problem on bad fluidity of molten iron caused by chrome in nickel and chrome ores. Limestone can not only provide alkalinity, but also can balance the above two additives. The metallurgical method of one-step blast-furnace smelting provided by the present invention is characterized by short technical process, high yield of continuous production, total extraction of nickel, chrome and iron in laterite nickel ore once for all, high ratio of resource utilization. The slag obtained by smelting is an excellent raw material to produce concrete, except the exhaustion of a given mass of CO₂ gas, no other solid or liquid wastes are produced and there is no pollution.

By contrast, the metallurgical technology of blast-furnace smelting provided by the present invention has some advantages, for example low cost. Blast furnace in the technology provided by the present invention can consume 150-200 kilowatt-hours per ton iron, while the conventional ore smelting technology need consume 2000-4000 kilowatt-hours and coke of 0.5 ton per ton iron; For example economic resources, high yield, namely the mean yield of blast furnace is bigger than that of ore-smelting furnace; such as little pollution, little dust, high recovery rate of the raw materials which are respectively 97 ∼ 98% for iron, 99% for nickel and 40 ∼ 50% for chrome.

### Specific embodiment:

The present invention can further be explained and described in combination with specific examples below.

Raw ores in examples are selected from nickel and chrome iron ores imported form Albania.

Crushing and sieving raw ores, mixing the feed of ore powder in grain diameter smaller than 2 mm thereof with coke powder, calcium lime/limestone and sintering to obtain sintered ore blocks;

Crushing and sieving the sintered blocks obtained by first sintering by means of a sieve with openings in the range between 25 and 53 µm (300-500 meshes) and then magnetic sorting to obtain refined ore powder.

Mixing the feed of the refined ore powder with coke powder, calcium lime/limestone and sintering to obtain sintered ore blocks.

Mixing sintered ore of the sintered ore blocks in particulate diameter of 10-50 mm with other raw materials and smelting to obtain ferronickel.

The main components in used nickel and chrome iron ore and its content (wt.%) are:

| components | Fe | Ni | Cr | Ca | Si | Mg | Al |
|---|---|---|---|---|---|---|---|
| Series code | | | | | | | |
| 1 | 7.18 | 4.37 | 11.93 | 18.14 | 21.08 | 0.84 | 6.17 |
| 2 | 17.81 | 3.21 | 9.26 | 16.25 | 18.27 | 1.18 | 5.77 |
| 3 | 26.28 | 2.68 | 8.10 | 14.36 | 17.35 | 1.45 | 4.69 |
| 4 | 36.54 | 2.30 | 6.32 | 11.87 | 16.09 | 1.64 | 3.14 |
| 5 | 43.51 | 1.83 | 4.71 | 8.29 | 15.14 | 1.94 | 2.84 |
| 6 | 54.26 | 0.57 | 0.35 | 4.57 | 5.88 | 2.11 | 2.11 |

The main components in obtained sintered ore and its content (wt.%) are:

| components | Fe | Ni | Cr | Ca | Si |
|---|---|---|---|---|---|
| Series code | | | | | |
| 1 | 9.01 | 4.23 | 10.29 | 16.17 | 19.14 |
| 2 | 23.14 | 3.60 | 7.39 | 14.19 | 16.32 |
| 3 | 33.83 | 2.97 | 7.10 | 13.24 | 16.10 |
| 4 | 46.83 | 2.51 | 5.48 | 12.31 | 14.26 |
| 5 | 55.59 | 2.13 | 3.62 | 7.25 | 4.77 |
| 6 | 65.51 | 0.63 | 0.33 | 3.67 | 2.59 |

Constitution of the furnace materials (Weight: Kg) is shown in following table.

| Components | Sintered ore | coke | fluorite | dolomite | limestone/ calcium lime |
|---|---|---|---|---|---|
| Series code | | | | | |
| 1 | 1000 | 455 | 200 | 80 | 350 |
| 2 | 1000 | 415 | 170 | 70 | 300 |
| 3 | 1500 | 680 | 240 | 90 | 300 |
| 4 | 1500 | 625 | 150 | 75 | 150 |
| 5 | 2000 | 920 | 100 | 20 | 160 |
| 6 | 2000 | 830 | 6 | - | 80 |

Metallurgical technology parameters of blast furnace:

| items | Crucible diameter | Vent diameter | fan | Wind pressure |
|---|---|---|---|---|
| Type code | | | | |
| Capacity of blast furnace 36 m³ | 2.1 m | 75 mm | 230 m/s | 559.95 kPa (4200 mmHg) |
| Capacity of blast furnace 90 m³ | 2.9 m | 100 mm | 380 m/s | 613.28 kPa (4600 mmHg) |

The main components in the obtained nickel iron by smelting and its content (wt.%) are:

| components | Fe | Ni | Cr | S | P |
|---|---|---|---|---|---|
| Series code | | | | | |
| 1 | 48.26 | 15.10 | 33.11 | 0.060 | 0.061 |
| 2 | 52.31 | 10.59 | 23.10 | 0.059 | 0.060 |
| 3 | 64.58 | 8.32 | 22.38 | 0.058 | 0.059 |
| 4 | 75.51 | 5.98 | 13.36 | 0.059 | 0.062 |
| 5 | 85.29 | 3.24 | 7.09 | 0.057 | 0.057 |
| 6 | 93.46 | 0.92 | 0.63 | 0.061 | 0.058 |

## Claims

1. A metallurgical method of ferronickel production by blast-furnace smelting nickel oxide ore with crystal water containing from 0.5% to 4% by weight of nickel, from 0.3% to 12% by weight of chromium, and from 7% to 55% by weight of iron, wherein the said method of blast- furnace smelting mainly comprising the following steps:
Crushing and sieving raw ores, mixing the feed of ore powder in grain diameter smaller than 2 mm thereof with coke powder, calcium lime/limestone and sintering to obtain sintered ore blocks;
Mixing sintered ore blocks, coke, limestone/calcium lime, dolomite and fluorite and blast-furnace smelting to obtain ferronickel; wherein the weight ratio of the following additives to sintered ore is:
fluorite 0.3∼20%
dolomite 0.5∼8%
limestone/calcium lime 4∼35%.

2. The metallurgical method according to Claim 1, wherein the blast furnace smelting further comprising the following steps:
Crushing and sieving the sintered blocks obtained by first sintering by means of a sieve with openings in the range between 25 an 53 µm (in 300-500 meshes) and then producing refined ore powder by magnetic sorting; Mixing the feed of the refined ore powder with coke powder, calcium lime/limestone and sintering to obtain sintered ore blocks;
Mixing the sintered ore blocks obtained by second sintering with coke, lime/limestone, dolomite and fluorite, and then blast-furnace smelting to obtain ferronickel.

3. The metallurgical method according to Claim 1 or 2, wherein the preferable weight ratio of the said additives to the sintered ore is:
fluorite 0.3∼10%
dolomite 0.5∼5%
limestone/calcium lime 8∼20%.

4. The metallurgical method according to Claim 1 or 2, wherein the content of CaO in the limestone is greater than 50% ,while that of CaO in calcium lime is greater than 80%.

5. The metallurgical method according to Claim 1 or 2, wherein the content of Mg in the dolomite is higher than 10%.

6. The metallurgical method according to Claim 1 or 2, wherein the content of CaF₂ in the fluorite is bigger than 80%.

## Patentansprüche

1. Metallurgisches Verfahren der Ferronickel-Produktion durch Verhütten von Nickeloxid-Erz mit Kristallwasser, das 0,5 Gewichts-% bis 4 Gewichts-% Nickel, 0,3 Gewichts-% bis 12 Gewichts-% Chrom und 7 Gewichts-% bis 55 Gewichts-% Eisen enthält, im Hochofen, worin das Verfahren des Verhüttens im Hochofen hauptsächlich die folgenden Schritte umfaßt:
Zerkleinern und Sieben von Roherzen, Mischen der Beschickung von Erz-Pulver mit einem Korn-Durchmesser von kleiner 2 mm mit Koks-Pulver, Calciumoxid/Kalkstein und Sintern unter Erhalt gesinterter Erz-Blöcke;
Mischen von gesinterten Erz-Blöcken, Koks, Kalkstein/Calciumoxid, Dolomit und Fluorit und Verhütten im Hochofen unter Erhalt von Ferronickel, worin der Gewichtsanteil der folgenden Additive zu gesintertem Erz wie folgt ist:
Fluorit: 0,3 bis ca. 20 %;
Dolomit: 0,5 bis ca. 8 %;
Kalkstein/Calciumoxid: 4 bis ca. 35 %.

2. Metallurgisches Verfahren nach Anspruch 1, worin das Verhütten im Hochofen weiter die folgenden Schritte umfaßt:
Zerkleinern und Sieben der gesinterten Blöcke, die durch den ersten Sinter-Schritt erhalten wurden, mittels eines Siebes mit Öffnungen im Bereich zwischen 25 und 53 µm (300 bis 500 mesh) und anschließendes Produzieren eines verfeinerten Erz-Pulvers durch Magnet-Scheiden; Mischen der Beschickung des verfeinerten Erz-Pulvers mit Koks-Pulver, Calciumoxid/Kalkstein und Sintern unter Erhalt gesinterter Erz-Blöcke;
Mischen der gesinterten Erz-Blöcke, die in dem zweiten Sinter-Schritt erhalten wurden, mit Koks, Calciumoxid/Kalkstein, Dolomit und Fluorit und anschließendes Verhütten im Hochofen unter Erhalt von Ferronickel.

3. Metallurgisches Verfahren nach Anspruch 1 oder 2, worin der bevorzugte Gewichtsanteil der Additive zu dem gesinterten Erz wie folgt ist:
Fluorit: 0,3 bis ca. 10 %;
Dolomit: 0,5 bis ca. 5 %;
Kalkstein/Calciumoxid: 8 bis ca. 20 %.

4. Metallurgisches Verfahren nach Anspruch 1 oder 2, worin der Gehalt an CaO in dem Kalkstein größer ist als 50 %, während der Gehalt an CaO in dem Calciumoxid größer ist als 80 %.

5. Metallurgisches Verfahren nach Anspruch 1 oder 2, worin der Gehalt an Mg in dem Dolomit höher ist als 10 %.

6. Metallurgisches Verfahren nach Anspruch 1 oder 2, worin der Gehalt an CaF₂ in dem Fluorit größer ist als 80 %.

## Revendications

1. Procédé métallurgique de production de ferronickel par fusion en haut-fourneau de minerais nickelifères oxydés avec de l'eau de cristallisation contenant de 0,5% à 4% en poids de nickel, de 0,3% à 12% en poids de chrome, et de 7% à 55% en poids de fer, où ledit procédé par fusion en haut-fourneau comprend essentiellement les étapes suivantes :
broyer et tamiser des minerais brutes, mélanger l'amenée de poudre de minerais d'un diamètre de grain inférieur à 2mm de ceux-ci avec une poudre de coke, chaux riche en calcium/calcaire et le fritter pour obtenir des blocs de minerais frittés ;
mélanger les blocs de minerais frittés, le calcaire/chaux riche en calcium, dolomite et fluorite et faire fondre dans le haut-fourneau pour obtenir du ferronickel ; où le rapport pondéral des additifs suivants au minerai fritté est :
fluorite 0,3-20%
dolomite 0,5-8%
calcaire/chaux riche en calcium 4~35%.

2. Procédé métallurgique selon la revendication 1, dans lequel la fusion en haut-fourneau comprend en outre les étapes suivantes :
broyer et tamiser les blocs frittés obtenus par le premier frittage au moyen d'un tamis avec des ouvertures dans la plage entre 25 et 53 µm (dans 300-500 mailles) et produire ensuite une poudre de minerai raffinée par triage magnétique ; mélanger l'amenée de la poudre de minerai raffinée avec la poudre de coke, chaux riche en calcium/calcaire et fritter pour obtenir les blocs de minerai frittés ;
mélanger les blocs de minerai frittés obtenus par le deuxième frittage avec le coke, la chaux/calcaire, dolomite et fluorite, et ensuite faire fondre dans le haut-fourneau pour obtenir du ferronickel.

3. Procédé métallurgique selon la revendication 1 ou 2, dans lequel le rapport pondéral préférable desdits additifs au minerai fritté est :
fluorite 0,3-10%
dolomite 0,5-5%
calcaire/chaux enrichie en calcium 8~20%.

4. Procédé métallurgique selon la revendication 1 ou 2, dans lequel la teneur en CaO dans le calcaire est supérieure à 50%, alors que celle de CaO dans la chaux riche en calcium est supérieure à 80%.

5. Procédé métallurgique selon la revendication 1 ou 2, dans lequel la teneur en Mg dans la dolomite est supérieure à 10%.

6. Procédé métallurgique selon la revendication 1 ou 2, dans lequel la teneur en CaF₂ dans la fluorite est supérieure à 80%.
